

1

2,840,468

## NOVEL GOLD ALLOYS AND POTENTIOMETER WIRES PRODUCED FROM THEM

Bert Brenner, Tenafly, N. J., assignor to Sigmund Cohn Corp., Mount Vernon, N. Y., a corporation of New York

No Drawing. Application February 4, 1958  
Serial No. 713,099

7 Claims. (Cl. 75—165)

The present application is a continuation-in-part of my copending application, Serial No. 607,976, filed September 5, 1956, now abandoned, which is in turn a continuation-in-part of my prior application, Serial No. 524,279, filed July 25, 1955, now abandoned, which is in turn a continuation-in-part of my application, Serial No. 441,627, filed July 6, 1954, now abandoned.

The present invention relates to novel gold alloys and to novel and improved potentiometer resistance elements and wires prepared from these alloys. These potentiometer resistance elements or wires are ideally suited for the construction of potentiometers, including those delicate potentiometers employed in telemetering devices, electronic computers and the like, as in electromechanical transducers employed to translate motion into changes of electrical characteristics.

In the construction of delicate and precise potentiometers and variable resistors it is very important if desirable results are to be obtained that the resistance element or wire employed have a low or controllable temperature coefficient of resistance, i. e., the variation in resistance should be small when the element or wire is subjected to temperature changes. The temperature coefficient of resistance is preferably as close to 0 p. p. m. as possible and desirably less than  $\pm 30$  p. p. m. as measured over the fundamental temperature interval of 0° to 100° C. The resistance element should have as high a resistivity as possible for many applications. It is also important that the resistance element or wire be easily workable and have a high tensile strength so that it can be drawn into an extremely fine wire and can be readily wound to form a variable resistance unit without danger of breaking. In addition, the resistance element or wire should be hard and it should not be subject to excessive wear when used in conjunction with a sliding metal contact brush, so as to provide a long operational life. It should also have electrical stability so that electrical characteristics will not "drift" with the passage of time nor with exposure to abnormal temperatures, and the alloy should resist oxidation and atmospheric corrosion.

Another important prerequisite of such resistance elements or wires is freedom from "noise" when used in a sensitive potentiometer or the like. "Noise" results in part from sharp random voltage or resistance peaks which are generated as the slider contact surface traverses the resistance windings of the potentiometer. The "noise" is much more pronounced with wires made of certain metals and alloys than with others. The preferred alloys of the present invention provide relative freedom from "noise."

Many attempts have been made to produce potentiometer resistance elements and wires, and alloys from which to make them, which have all of the hereinabove mentioned properties. I have succeeded in producing alloys of gold which will impart these properties to a potentiometer resistance element or wire made from such alloys.

It is an object of the present invention to provide novel

2

alloys of gold, and potentiometer resistance elements and wire prepared from said alloys, which will have substantially all of the hereinabove mentioned desirable properties.

5 It is another object of the invention to provide novel potentiometer resistance elements or wires which have optimum electrical, physical and chemical properties, including low temperature coefficients of resistance.

Other objects and advantages of this invention will be apparent to those skilled in the art from the description which follows.

In accordance with my invention I have discovered that alloys, composed primarily of gold (desirably between about 50% and 89.5%), with between about 6% and 15 12% of chromium along with a metal of the first triad of group VIII of the periodic chart totaling at least about 75% of the chromium concentration and from 6% up to about 30% of the alloy, provide potentiometer wires and resistance elements which have a low temperature coefficient of resistance, high electrical resistance and workability as well as other properties which make them satisfactory for resistance wires and elements. The gold concentration in all cases shall constitute substantially the difference between the total concentration of the other metals and 100%.

20 The preferred alloys of the invention have the following composition:

Chromium ..... 6% to 12%

30 Metals of the first triad of group VIII of the periodic chart ..... 22% to 30%, more preferably 24% to 30%

Gold ..... remainder (but desirably 60% to 35 70 or 72%)

An alloy in accordance with the present invention containing 10% chromium, 25% nickel and 65% gold is the most satisfactory alloy produced to date. Potentiometer wires produced from it have no measurable "noise" and have excellent life, are easily drawn and not brittle, and have a low temperature coefficient of resistance.

40 The metals of the first triad of group VIII of the periodic chart are a well-known class which includes nickel, iron and cobalt. These metals have an atomic number of from 26 to 28 and are known as the "transitional elements." The concentration of the metals of this class in the alloys of the invention may consist of a single metal or two or three metals of the group. Nickel is the preferred metal of the group.

50 I prefer to incorporate into the alloys of my invention small amounts of an element more electronegative than nickel and chromium, to act as a deoxidizer or degasifier. Such other element or elements include, but are not limited to, carbon, manganese, aluminum, zirconium, thorium, titanium and beryllium. Manganese and aluminum are preferred. The desirable concentration of these elements is from about 0.001% to 1% of the alloy, although 0.2% is sufficient.

The alloys of the present invention may be prepared 60 in accordance with the following process.

A high frequency induction furnace is satisfactory for the melting of the alloy. The melting of the components of the alloy may take place in a zirconium silicate crucible. The gold is melted first. A neutral flux is then added in sufficient quantity to cover the molten gold. Dry barium chloride is a satisfactory flux. One or more metals of the first triad of group VIII of the periodic chart and the chromium are then added until a uniform melt is obtained. The deoxidizer or other element is then added in slightly greater amounts than desired for the finished alloy to compensate for oxidation losses during melting

and pouring. The melt is then poured into an ingot mold, immediately remelted, and additional small amounts of deoxidizer or other element added, and the melt is again poured into an ingot mold. The alloy ingot is cold rolled to about half its original diameter.

Following the cold rolling of the ingot, I anneal it in an inert or reducing atmosphere, such as nitrogen or hydrogen gas, for about 15 minutes at 1,200° F. Rolling is repeated and until the ingot is reduced to a diameter of about 0.06 inches, with annealing treatments as necessary to impart ductility. The alloy is then reduced into wire of the desired diameter by drawing it through diamond dies in accordance with the usual wire-drawing techniques. Where necessary during the drawing process, the wire is heat treated to relieve any stresses. When reduced to the required diameter, the wire is again heat treated, enameled if necessary, and is then suitable for use in manufacturing rheostats and potentiometers, etc. No intricate baking step is required to stabilize the temperature coefficient of resistance of the wire or wound coil. The required stable electrical characteristics are produced in the present invention by means of varying the initial composition of the alloy.

In order more clearly to disclose the nature of the present invention, specific examples illustrating the present invention will hereinafter be described. It should be understood, however, that this is done solely by way of example and is intended neither to delineate the scope of the invention nor limit the ambit of the appended claims. In each example the alloys, and the potentiometer wires produced from the alloys, are obtained in accordance with the hereinabove described process. In each of the examples, the temperature coefficient of resistance was measured over the fundamental temperature range between 0° and 100° C. and was found to be about  $\pm 30$  p. p. m. or less in each case.

#### Example 1

The alloy was produced by melting sufficient quantities of metals to produce the following composition:

|          | Percent |
|----------|---------|
| Gold     | 65      |
| Chromium | 10      |
| Nickel   | 25      |

Sufficient manganese was added to constitute an additional 0.2% of the alloy and the alloy drawn into a fine potentiometer wire. This alloy is the preferred alloy of the invention and provides potentiometer resistance wire of optimum properties, including no significant noise, a temperature coefficient of resistance of 10 p. p. m., and a resistivity of 550 ohms/c. m. f.

#### Example 2

The alloy was produced by melting sufficient quantities of metals to produce the following composition:

|          | Percent |
|----------|---------|
| Gold     | 70      |
| Chromium | 10      |
| Nickel   | 20      |

Sufficient manganese was added to constitute an additional 0.2% of the alloy and the alloy drawn into a fine potentiometer wire. This alloy has a resistivity of 615 ohms/c. m. f.

#### Example 3

The alloy was produced by melting sufficient quantities of metals to produce the following composition:

|          | Percent |
|----------|---------|
| Gold     | 70      |
| Chromium | 6       |
| Nickel   | 24      |

Sufficient manganese was added to constitute an additional

0.2% of the alloy and the alloy drawn into a fine potentiometer wire. The alloy has a resistivity of 450 ohms/c. m. f.

#### Example 4

The alloy was produced by melting sufficient quantities of metals to produce the following composition:

|          | Percent |
|----------|---------|
| Gold     | 58      |
| Chromium | 12      |
| Nickel   | 30      |

Sufficient manganese was added to constitute an additional 0.2% of the alloy and the alloy drawn into a fine potentiometer wire. The alloy has a resistivity of 620 ohms/c. m. f.

#### Example 5

The alloy was produced by melting sufficient quantities of metals to produce the following composition:

|          | Percent |
|----------|---------|
| Gold     | 89      |
| Chromium | 6       |
| Nickel   | 15      |

Sufficient manganese was added to constitute an additional 0.2% of the alloy and the alloy drawn into a fine potentiometer wire. The alloy has a resistivity of 490 ohms/c. m. f.

Potentiometer wires or elements according to the present invention may be employed in rheostats, potentiometers and variable resistors of many types, including the low torque toroidal resistor described in my U. S. Letters Patent No. 2,537,733, granted January 9, 1951.

The term "potentiometer wire," as used throughout this application, is intended to include wire and other suitable forms of potentiometer resistance elements. The wires may take the form of various shapes, including flat strips and the more conventional filaments of round cross-section.

Percentages of materials are expressed in terms of percent by weight.

The terms and expressions which I have employed are used as terms of description and not of limitation, and I have no intention, in the use of such terms and expressions, of excluding any equivalents of the features shown and described or portions thereof, but recognize that various modifications are possible within the scope of the invention claimed.

What is claimed is:

1. A gold alloy comprising between about 6% and 12% chromium, nickel in an amount of between about 22% and 30%, the remainder of the alloy being substantially gold which constitutes between about 50% and 72% of the alloy.
2. A gold alloy comprising between about 6% and 12% chromium, nickel in an amount of between about 24% and 30%, the remainder of the alloy being substantially gold which constitutes between about 60% to 70% of the alloy.
3. A gold alloy consisting essentially of about 25% nickel, 10% chromium and 65% gold.
4. A gold alloy as defined by claim 2, which also contains an amount of an element more electronegative than nickel and chromium which constitutes up to about 1% of the alloy, said more electronegative element being a member selected from the class consisting of carbon, manganese, aluminum, zirconium, thorium, titanium and beryllium.
5. A potentiometer having as a component a wire winding comprising a gold alloy in which gold constitutes the major proportion of the alloy, and which also contains between about 6% and 12% chromium and nickel in an amount of at least 75% of the chromium content and from about 6% up to about 30% of the alloy.

6. A potentiometer having as a component a wire winding comprising a gold alloy comprising between about 6% and 12% chromium, nickel in an amount of at least about 75% of the chromium concentration and from about 6% to about 30%, the remainder of the alloy being substantially gold which constitutes between about 60% to 80% of the alloy.

7. A potentiometer having as a component a wire winding comprising an alloy consisting essentially of about 20% nickel, 10% chromium and 70% gold. 10

## References Cited in the file of this patent

## UNITED STATES PATENTS

|           |        |       |               |
|-----------|--------|-------|---------------|
| 1,562,958 | Hansen | ----- | Nov. 24, 1925 |
| 2,042,972 | Thomas | ----- | June 2, 1936  |

## FOREIGN PATENTS

|         |               |       |               |
|---------|---------------|-------|---------------|
| 254,979 | Great Britain | ----- | July 14, 1926 |
|---------|---------------|-------|---------------|